



US005499938A

# United States Patent [19]

Nakamoto et al.

[11] Patent Number: 5,499,938

[45] Date of Patent: Mar. 19, 1996

[54] FIELD EMISSION CATHODE STRUCTURE, METHOD FOR PRODUCTION THEREOF, AND FLAT PANEL DISPLAY DEVICE USING SAME

[75] Inventors: **Masayuki Nakamoto; Tomio Ono; Tadashi Sakai**, all of Yokohama, Japan

[73] Assignee: **Kabushiki Kaisha Toshiba**, Kanagawa, Japan

[21] Appl. No.: 291,937

[22] Filed: Aug. 16, 1994

## Related U.S. Application Data

[63] Continuation-in-part of Ser. No. 38,936, Mar. 29, 1993, abandoned.

## Foreign Application Priority Data

Jul. 14, 1992 [JP] Japan ..... 4-186753  
Aug. 17, 1993 [JP] Japan ..... 5-203167  
Dec. 27, 1993 [JP] Japan ..... 5-332043

[51] Int. Cl. <sup>6</sup> ..... H01J 9/02

[52] U.S. Cl. ..... 445/50

[58] Field of Search ..... 445/24, 50, 49

## References Cited

### U.S. PATENT DOCUMENTS

4,307,507 12/1981 Gray et al. ..... 437/228  
4,721,885 1/1988 Brodie ..... 313/576  
5,038,070 8/1991 Bardai et al. ..... 313/309  
5,140,219 8/1992 Kane ..... 313/495  
5,166,709 11/1992 Kubelik ..... 346/155  
5,221,221 6/1993 Okaniwa ..... 445/24  
5,254,137 6/1993 Mitani ..... 29/25.03  
5,270,258 12/1993 Yoshida ..... 445/50

### FOREIGN PATENT DOCUMENTS

160740 12/1981 Japan ..... 445/50  
615780 2/1980 Switzerland .

## OTHER PUBLICATIONS

Spindt et al., "Physical Properties of Thin-Film Field Emission Cathodes With Molybdenum Cones," Journal of Applied Physics 47(12):5248-5263 (1976).

M. Sokolich et al., "Field Emission From Submicron Emitter Arrays," Technical Digest of the International Electron Devices Meeting 1990, San Francisco, CA, Dec. 9-12, 1990, pp. 159-162.

Primary Examiner—Kenneth J. Ramsey  
Attorney, Agent, or Firm—Finnegan, Henderson, Farabow, Garrett & Dunner

## ABSTRACT

A field emission cathode which comprises an emitter provided with a sharp point for emission of electrons and a controlling gate electrode is composed of a supporting substrate, an emitter material layer formed of an emitter material, superposed on and attached fast to the supporting substrate, and provided with an emitter hole, an insulator layer so formed on the surface of the emitter material layer as to expose the tip part of the emitter projection therethrough, and an impurity diffusion layer formed on the surface of the insulator layer and enabled to function as an etching stopper layer. The method for the production of the field emission cathode comprises a step of forming a first hole pointed toward the leading end thereof on a first supporting substrate, a step of forming the impurity diffusion layer on the surface of the first supporting substrate, a step of forming the insulator layer on the surface of the impurity diffusion layer, a step of depositing an emitter material layer on the surface of the insulator layer including a hole while filling the hole with an emitter material thereby giving rise to a laminate, a step of integrally joining a second supporting substrate to the surface of the emitter material layer of the laminate, a step of removing by etching the first supporting substrate thereby exposing the surface of the impurity diffusion layer including the projection corresponding to the first hole, and a step of selectively removing the impurity diffusion layer and the insulator layer thereby exposing a tip of the projection of the emitter layer.

16 Claims, 12 Drawing Sheets



**FIG. 1a****FIG. 1b****FIG. 1c****FIG. 1d****FIG. 1e****FIG. 1f****FIG. 1g****FIG. 1h**

FIG. 2



FIG. 3



FIG. 4



FIG. 5



FIG. 6



FIG. 7a



FIG. 7b



FIG. 7c



FIG. 7d



FIG. 8



FIG. 9a



FIG. 9b



FIG. 9c



FIG. 10



**FIG. 11a****FIG. 11b****FIG. 11c****FIG. 11d**

**FIG. 11e****FIG. 11f****FIG. 11g****FIG. 11h**

**FIG. 12a****FIG. 12b****FIG. 12c****FIG. 12d****FIG. 12e****FIG. 12f**

**FIG. 13a****FIG. 13b****FIG. 13c****FIG. 13d****FIG. 13e****FIG. 13f**

**FIG. 14a****FIG. 14b****FIG. 14c****FIG. 14d****FIG. 14e****FIG. 14f**

**FIELD EMISSION CATHODE STRUCTURE,  
METHOD FOR PRODUCTION THEREOF,  
AND FLAT PANEL DISPLAY DEVICE USING  
SAME**

This is a continuation-in-part of application Ser. No. 08/038,936 filed Mar. 29, 1993 now abandoned.

**BACKGROUND OF THE INVENTION**

The present application claims priority of Japanese Patent Application No. Hei-4-186753 filed on Jul. 14, 1992, Japanese Patent Application No. Hei-5-203167 filed on Aug. 27, 1993 and Japanese Patent Application No. Hei-5-332043 filed on Dec. 17, 1993.

**FIELD OF THE INVENTION AND RELATED  
ART STATEMENT**

This invention relates to a field emission cathode structure, a method for the production thereof, and a flat panel display device using the cathode.

In recent years, the advanced technology on the fabrication of Si semiconductors has been lending itself immensely to the development of field-emission type cathode structures and to the utilization of these cathodes in ultraspeed microwave devices, power devices, electron beam devices, flat panel display devices, etc. As a typical example of the cathode, what has been reported by C. A. Spindt et al. in Journal of Applied Physics, Vol. 47, No. 12, December 1976, pages 5248-5263 has been known to the art.

The field emission cathode structure disclosed therein, as illustrated in FIG. 9a, FIG. 9b, and FIG. 9c of the present specification, is produced by forming a  $\text{SiO}_2$  layer 2 as an insulating layer by the technique of deposition such as CVD on a Si single crystal substrate 1, further forming thereon a Mo layer 3 destined to serve as a gate electrode layer as by the electron beam vacuum deposition technique, boring a pinhole 5 approximately 1.5  $\mu\text{m}$  in diameter through the layers 2 and 3 by means of etching, then forming an Al layer 4 destined to serve as a separating layer by means of vacuum deposition [FIG. 9a], vacuum depositing thereon a metal such as Mo which is destined to form an emitter as by the technique of electron beam vacuum deposition while keeping the Si single crystal substrate 1 in rotation thereby giving rise to a conical pile of Mo inside the pinhole 5 by utilizing the phenomenon that the diameter of the pinhole 5 converges in proportion as the deposition of Mo proceeds [FIG. 9b], and finally finishing a conical emitter 7 by peeling the Al separating layer 4 and removing the Mo layer 6 [FIG. 9c].

The electronic device using a cathode structure such as, for example, the flat panel display device is constructed by causing a Si single crystal substrate 1 having a multiplicity of such cathodes superposed thereon to be opposed across a prescribed interval to a glass face plate 8 having a phosphor layer superposed thereon as illustrated in FIG. 10. In this diagram, A stands for a region for the formation of cathodes. This flat panel display device using field emission cathodes is different from the display device using a liquid crystal in being a luminescent type. It obviates the necessity for using a back light and consequently promises a saving in power consumption. Owing to these features, it has been attracting keen attention.

The conventional method for producing the field emission cathode system, the field emission cathode structure obtained by the method, and the electronic devices using

such cathode structures, however, entail the following important problems.

Firstly, in the conventional method for rotary vacuum deposition described above, since the formation of the emitter 7 inside the pinhole 5 is attained by utilizing the phenomenon that the diameter of the pinhole 5 bored in the Mo layer 3 gradually converges, the height of the emitter and the shape of the tip of the emitter are liable to loss of consistency. The cathode structure which is obtained by this method, therefore, produces field emission with poor uniformity and lacks the sharpness of the tip of the emitter which is necessary for improving the efficiency of field emission and, as a result, entails such problems as decline of the efficiency of field emission and growth of power consumption. Further, the fact that the reproducibility of shape and the yield of production are both inferior gives rise to a problem of extremely high cost of production in the fabrication of a multiplicity of field emission cathode structures on one and the same substrate.

Secondly, since the  $\text{SiO}_2$  insulating layer is formed by the technique of CVD, the distance between the gate and the emitter on which the efficiency of field emission heavily hinges defies accurate control, and the magnitudes of field emission which the plurality of cathode structures severally generate lack uniformity. In the production of a flat panel display device, for example, the picture elements corresponding to the individual cathode structures are suffered to betray inconsistency of luminance. As respects the flat panel display device, owing to the slight loss of consistency in the distance between the gate and the emitter and in the shape of the tip of the emitter, it often happens that the ratio of the current of electrons between the gate and the emitter to the current of electrons between the anode and the emitter increases. There are times when the current of electrons between the gate and the emitter even reaches 60% of the total current of electricity. Thus, the problem arises that the efficiency of light emission of the picture elements (fluorescent elements) corresponding to the individual cathode structures is degraded and, at the same time, the picture elements suffer from serious inconsistency in luminance.

Thirdly, the size of the Si single crystal substrate imposes a limit on the regions to be used for the formation of field emission cathode structures or the number of such cathode structures to be formed and, at the same time, impairs the productivity of the cathode structures. This fact implies that the flat panel display device using a multiplicity of cathode structures is limited in size. Further, the flat panel display device by nature is fated to use the Si single crystal substrate as part of the housing of the device. As a vacuum container, the housing is conspicuously deficient in strength. Especially, when the image screen grows in size, the housing retains required strength only with increasing difficulty.

Fourthly, since the emitter is formed by depositing the Si single crystal substrate or conductive substrate concurrently serving as a cathode, the continuity between the emitter and the cathode is disrupted along their interface no matter whether the material for the emitter and that for the cathode are different or same. Thus, the disadvantage arises that the emitter will peel and incur loss of resistance and, consequently, generate heat possibly to the extent of deteriorating the emitter itself.

For the sake of eliminating the limit on size and enhancing the strength of the housing, an idea of superposing the Si single crystal substrate fast on a structural substrate such as a glass substrate may be conceived. The mere superposition results in an addition to the thickness of the cathode part and

proves unfit for such electronic devices which are directed toward decreasing weight and thickness, for example. The substitution of a glass substrate for the Si single crystal substrate indeed eliminates the problems on size mentioned above. It, however, necessitates formation of a conductive layer on the glass substrate for the purpose of ensuring maintenance of conductivity to the emitter. Thus, the formation of the  $\text{SiO}_2$  insulating layer does not permit adoption of the technique of CVD but requires use of the technique of electron beam vacuum deposition or the technique of sputtering. The  $\text{SiO}_2$  insulating layer which is obtained by such a technique, however, assumes a more porous texture and contains more pinholes than the layer obtained by the technique of CVD and suffers from aggravated inconsistency in the distance between the gate and emitter which governs the efficiency of field emission.

The flat panel display device using the conventional field emission cathode structures entails the following problems in addition to the problems pertaining to the process of manufacture of cathode structures mentioned above. When the field emission cathode structures are used, in spite of an increase in the voltage applied between the cathode and the anode to a level of about 100 V, the energy of the electron beam is small as compared with that of the ordinary C-CRT and the fluorescent elements collect electric charge on their surfaces possibly to the extent of repelling the electron beam. Thus, the problem arises that the infiltration of electrons in the fluorescent elements occurs only to several nm from their surfaces and the fluorescent elements suffer from poor efficiency of emission. When the applied voltage is increased, the energy of the electron beam is augmented and the efficiency of emission is enhanced and, at the same time, the practicability of allowing use of fluorescent elements which avoid inducing saturation of luminance and excel in efficiency of emission is realized. The increased voltage, however, entails such problems as ionization of impurity gas and consequent sputtering of the surface of the cathode and breakdown of the insulation between the gate and the cathode. Since these circumstances compel the applied voltage lower than that normally used in the C-CRT, the efficiency of emission which is actually obtained is lower than that which is obtained inherently.

As a way of compensating, if only nominally, this decline of the luminous efficiency, the method which consists in coating the surface of the fluorescent face plate opposite the surface thereof intended for observation, namely the fluorescent rear surface, with aluminum thereby forming a so-called metal back and enabling the metal back to reflect the light radiated on the fluorescent rear surface side toward the observation surface side may be cited. This method has found extensive utility in the ordinary C-CRT devices. The use of the metal back, however, necessitates application of a high voltage even reaching the range from 6,000 V to 8,000 V for enabling the electron beam to pass through the Al layer and, consequently, entails the aforementioned problems of sputtering and breakdown of the cathode, and renders it extremely difficult to maintain mutual insulation of the anode and the cathode because the gap intervening between them is as narrow as to fall in the range of from several  $\mu\text{m}$  to 1 mm.

As described above, the method for the production of the conventional field emission cathode structure poses various problems such as degradation and inconsistency of the efficiency of field emission and inferiority of the yield of production owing to the marked deficiency of the shape of the emitter in reproducibility and uniformity and, at the same time, entails such problems as restriction of the region for

the formation of the field emission cathode structure by the size of the Si single crystal substrate and inevitable use of the Si single crystal substrate as part of the housing of the device.

With a view to improving the reproducibility and uniformity of the shape of emitter, Sokolich et al. (IEDM 90, pages 159-162) have developed a method for arranging uniform tips on a polysilicon substrate by forming in a  $\langle 100 \rangle$  Si single crystal substrate by the etching technique a pyramidal hole having a sharp bottom tip, forming on the surface of the hole a thin oxide film as an etching barrier, subsequently depositing polysilicon in the Si mold wafer, and further removing the mold wafer by etching. The polysilicon tips thus produced are coated as with Mo, overcoated with a  $\text{SiO}_2$  film by the CVD technique, further coated with a layer of grid metal, and then finished as field emission cathodes.

This method of manufacture proposed by Sokolich et al., however, has the following problems. When the mold layer is used, the tips are discernibly improved in reproducibility and uniformity as compared with those obtained by the rotary vapor deposition method described above. The sharpness of the tips does not necessarily deserve to be called sufficient, because of the difficulty of coating emitter material on the sharp emitter tips, and the emitter material coated on polysilicon is sometimes peeled off. Further, since the  $\text{SiO}_2$  film is formed by the CVD technique, the gaps intervening between the gates and the emitters defy control and permit no easy decrease. Thus, it has been difficult for this film to be produced in high quality.

As respects the flat panel display device which uses the conventional field emission cathode structure, even when the device is relieved of the problems which pertain to the emitter, it still entails such structural problems as inferior efficiency of emission (luminance) of picture elements and serious inconsistency of luminance.

#### SUMMARY OF THE INVENTION

This invention has been produced for the purpose of solving the problems of the prior art described above.

One object of this invention is to provide a method for the production of a field emission cathode structure which permits easy fabrication of emitters excelling in reproducibility and uniformity of shape, allows accurate control of the intervals between gates and emitters, enables the region for the formation of emitters to be easily increased in area without entailing any addition to the thickness of the cathode structure, and abounds in productivity.

Another object of this invention is to provide a field emission cathode structure which excels in efficiency and uniformity of electron emission and exhibits ample strength in the case that it is used as part of the housing of the device.

A further object of this invention is to provide a field emission cathode structure which incurs such adverse phenomena as separation and deterioration only sparingly.

Yet another object of this invention is to provide a flat panel display device which is adapted to improve the quality of the displayed image by augmenting the luminance of emission of the picture elements and, at the same time, curbing the inconsistency of luminance among the picture elements.

The first method of this invention for the production of a field emission cathode structure is characterized by comprising a step of providing a first substrate with holes with a sharp point, a step of forming an insulating layer on the

surface of the first substrate inclusive of the interiors of the holes, a step of forming an emitter material layer on the insulating layer while filling the interiors of the holes with the emitter material layer, a step of joining the first substrate with a second substrate formed of a structural substrate in such a manner as to have the emitter material layer interposed therebetween, a step of removing the first substrate by etching thereby exposing the insulating layer and, at the same time, allowing protrusions conforming to the part of the emitter material filling the interiors of the holes to thrust out, a step of forming a gate electrode layer on the exposed insulating layer, and a step of removing part of the insulating layer and gate electrode layer thereby forming an emitter.

The field emission cathode system of this invention is obtained by the method for production mentioned above, which field emission cathode system is characterized by comprising a structural substrate, an emitter material layer superposed fast on the structural substrate and provided with protruding emitters with a sharp point, an insulating layer formed on the emitter material layer in such a manner as to expose the points of the emitters, and a gate electrode layer formed along the shape of the emitters through the medium of the insulating layer and, at the same time, provided with opening parts encircling the points of the emitters.

The second method of this invention for the production of a field emission cathode structure comprises a step of first forming a first hole having a sharp pointed tip on a first main surface of a first supporting substrate, a step of forming a high-concentration impurity diffusion layer on the main surface of the impurity diffusion layer including the wall surfaces of the first hole, a step of forming an insulator layer on the surface the impurity diffusion layer including a second hole formed to cover the first hole, a step of forming a smooth emitter material layer surface on the surface of the insulator layer including a third hole formed to cover the second hole and meanwhile filling the third hole with an emitter material, a step of integrally joining a second supporting substrate to the surface of the emitter material layer, a step of removing by etching the first supporting substrate and exposing the impurity diffusion layer including the projection corresponding to the first hole, and a step of selectively removing the impurity diffusion layer and the insulator layer in the tip part of the projection thereby exposing the tip part of the projection formed of the emitter material.

The field emission cathode according to the second method comprises a supporting substrate, an emitter material layer formed on the surface of the supporting substrate and provided with an emitter projection having a sharp pointed tip, an insulator layer formed on the emitter material layer and adapted to expose the tip part of the emitter projection, and a high-concentration impurity diffusion layer formed on the insulator layer and adapted to expose the tip part of the emitter projection.

The field emission cathode according to the second method has originated in the interest drawn to the fact that a pyramidal or conically hole having a sharp pointed tip can be formed on the surface of a supporting substrate such as, for example, a Si single crystal substrate by harnessing the anisotropy of etching, the fact that a layer having an impurity diffused therein functions as an etching stopper layer, the fact that the impurity diffusion layer also functions as a gate electrode layer depending on the magnitude of resistance thereof, and the fact that an oxide layer (insulator layer) having a sharp pointed tip part is formed along a prescribed surface by the use of the thermal oxidation method.

In the field emission cathode and the method for the production thereof contemplated by the present invention,

the first supporting substrate may be made of any material which satisfies the condition that it should permit a hole of a sharp pointed tip to be selectively formed therein and exhibit a selective etching property with respect to an insulating layer and a high-concentration impurity diffusion layer to be integrally joined thereto. It is, however, desired to be a Si or Ge single crystal substrate in due respect of the ease with which the high-concentration impurity diffusion layer is formed and the ease with which the formation of an insulator layer rich in accuracy of film thickness and shape is controlled.

Silicon (Si) containing boron (B) as a p-type impurity at a concentration of not less than  $3 \times 10^{19} \text{ cm}^{-3}$  may be cited as one example of the material for the high-concentration impurity diffusion layer. When the concentration of this impurity is as high as about  $10^{20}$  to  $10^{21} \text{ cm}^{-3}$ , the high-concentration impurity diffusion layer can be used concurrently as a gate electrode layer because the electric resistance is as low as about  $10^{-4} \Omega \cdot \text{cm}$ . It should be noted, however, that the material for the impurity diffusion layer does not need to be limited to the particular substance mentioned above. It is only required to be such that the impurity diffusion layer may function as an etching stopper layer when the first supporting substrate is removed by etching. It may be an n-type material or an i-type material instead of the p-type material mentioned above.

Further, the insulator layer may be formed by depositing  $\text{SiO}_2$  on the surface of the impurity diffusion layer mentioned above by the use of the CVD method, for example. The insulator layer, however, is desired to be formed by subjecting the surface of the impurity diffusion layer mentioned above to the process of thermal oxidation because this process imparts a dense texture to the produced layer and permits easy control of the thickness of the layer and allows the insulator layer having a sharp pointed tip to be formed along the wall surfaces of a pyramidal hole, for example.

In the method for the production of the field emission cathode according to this invention, since the high-concentration impurity diffusion layer destined to serve as an etching stopper layer and the insulator layer such as, for example, a thermally oxidized insulating layer are superposed on the surface of the first supporting substrate such as, for example, a Si single crystal substrate including the hole formed therein and the emitter material layer is subsequently superposed thereon, the thermally oxidized insulation layer can be formed as easily controlled and, therefore, the distance between the gate and the emitter can be controlled with high accuracy. Even when the insulator layer is formed in the smallest possible thickness for the purpose of closely approximating the gate and the emitter to each other, the supporting substrate can be removed by etching without exposing the insulator layer and the emitter material layer to the possibility of corrosion because the impurity diffusion layer functions as an etching stopper layer. Since the thermally oxidized insulation layer and the emitter material layer are protected against the corrosion by the etching liquid as described above and also since the distance between the gate and the emitter is decreased, the field emission efficiency and the uniformity of the field emission cathode are improved to a great extent.

Besides, since the emitter material is disposed as embedded (filled) in the hole formed in the supporting substrate and the hole is formed with high accuracy as well, the emitter which is uniform in height, shape, and sharpness of sharp pointed tip is manufactured with high repeatability. In the hole formed in the supporting substrate, the tip of the hole gains in sharpness because the growth of the thermally

oxidized insulation layer on the inner wall surfaces of the hole advances toward the interior of the hole. As a natural consequence, the tip part of the emitter formed by filling the emitter material in the hole becomes sharp (refer to FIG. 11b).

The high-concentration impurity diffusion layer primarily functions as an etching stopper layer. When it has a high p-type impurity concentration and enjoys high electric conductivity, it can be used directly as a gate electrode layer. When the etching stopper layer is concurrently used as a gate electrode layer, this layer and the insulator layer which has been formed as ideally controlled cooperate to permit accurate control of the distance between the gate and the emitter and the mutual approximation thereof and, at the same time, obviates the necessity of the step for the formation of the gate electrode layer. The omission of this step naturally results in reducing the labor, man-hour, and material cost involved in the production of the field emission cathode of this invention.

In addition to the first and the second methods, we will describe the other methods to which the above methods are applied. The third method is characterized by comprising a step of incising a hole having a sharp pointed bottom part on a first main surface side of a first supporting substrate, a step of forming an insulating layer on the first main surface of the first supporting substrate including the inner walls of the hole, a step of depositing an emitter material on the surface of the insulating layer while filling the emitter material in the hole thereby forming an emitter material layer provided with a projection having a sharp pointed tip, a step of joining a second supporting substrate to the surface of the emitter material layer opposite to the surface thereof on which the projection is formed thereby causing the second supporting substrate to support the emitter material layer, a step of removing by etching the first supporting substrate from the second main surface side thereof until at least the tip part of the insulating layer covering the projection of the emitter material layer is exposed, and until the end of a tip of the projection of the emitter material layer provided with the projection corresponding to the hole falls flush with the surface of the first supporting substrate after completion of the etching, and a step of progressively etching the insulating layer from the portion thereof exposed from the first supporting substrate thereby effecting selective removal by etching of the insulating layer, exposing the tip part of the projection of the emitter material layer previously covered by the insulating layer and consequently forming an emitter and, at the same time, allowing the first supporting substrate to remain at least in such a manner as to be opposed across a gap to the tip part of the emitter and forming a gate layer.

The fourth method is alternatively characterized by comprising a step of forming an etching stopper layer on a first main surface of a first supporting substrate, a step of incising on the first main surface side of the first supporting substrate a hole having a sharp pointed bottom part through the etching stopper layer to a depth reaching halfway along the thickness of the first supporting substrate, a step of forming an insulating layer on the etching stopper layer including the inner wall surfaces of the hole, a step of depositing an emitter material on the surface of the insulating layer while filling the emitter material in the hole thereby forming an emitter material layer provided with a projection having a sharp pointed tip, a step of removing by etching the first supporting substrate from the second main surface side of the substrate until the etching stopper layer thereby exposing the tip part of the insulating layer covering the projection of the emitter material layer through the surface of the etching

stopper layer, and a step of progressively etching the insulating layer from the portion thereof exposed through the etching stopper layer thereby selectively removing by etching the insulating layer, exposing the tip part of the projection of the emitter material layer previously covered by the insulating layer and forming an emitter and, at the same time, allowing the etching stopper layer to remain at least in such a manner as to be opposed across a gap to the tip part of the emitter and forming a gate layer.

In the method of this invention for the production of the field emission cathode structure, since the insulating layer is first formed on the first substrate provided with the holes and the emitter material layer is subsequently formed, the gaps between the gates and the emitters can be controlled with high accuracy. The emitters correspond to the parts of the emitter material filling the interiors of the holes formed in the first substrate. When the holes are accurately formed in advance, therefore, the emitters having a sharp point and excelling in height can be obtained with ideal reproducibility. When the insulating layer is formed of a thermally oxidized  $\text{SiO}_2$  layer, the points of the produced emitters have greater sharpness because the  $\text{SiO}_2$  layer is formed in a swelled state on the inner walls of the holes. These emitters are conspicuously improved in efficiency and uniformity of field emission. Since the emitter material layer is formed on the first substrate and joined to the structural layer and, thereafter, the first substrate which is no longer necessary is dissolved and removed, a multiplicity of first substrates having emitters formed thereon can be integrally formed on one structural substrate. As a result, the area for the formation of cathodes can be easily enlarged and, at the same time, the productivity of cathode structure can be enhanced. Further, the structural substrate can be maintained in a small thickness.

The flat panel display device of this invention is provided with a face plate having a phosphor layer and an anode electrode layer sequentially superposed therein and a field emission cathode plate opposed to the phosphor layer and fitted with a cathode electrode layer, emitters formed on the cathode electrode layer, and a gate electrode layer adapted to control the flows of electrons discharged from the emitters, which flat panel display device is characterized by having a second phosphor layer formed on the gate electrode layer around the emitters and/or in the emitter opening parts of the gate electrode layer.

In the flat panel display device of this invention, since the second phosphor layer is formed on the gate electrode layer around the emitters and/or in the emitter opening parts of the gate electrode layer, the currents of electrons flowing between the gates and the cathodes which generally make no contribution to the emission of light enable the second phosphor layers to emit light efficiently. The light thus emitted is reflected by the gates of a metallic substance. The gates, therefore, fulfill the function of a metal back. Thus, this light coupled with the light emitted from the fluorescent material on the gate electrode layer and the light emitted from the fluorescent material on the face plate enhances the efficiency of emission and the luminance of the emitted light. When the electric currents flowing between the anodes and the cathodes are deprived of consistency by changes in the distances between the gates and the cathodes and the distances between the cathodes and the anodes, the possible loss of consistency of the total amount of emitted light (inconsistency of luminance among picture elements) can be curbed by the light emitted from the phosphor layer formed on the gate electrode layer.

## BRIEF DESCRIPTION OF THE DRAWING

FIGS. 1a, 1b, 1c, 1d, 1e, 1f, 1g and 1h are cross sections illustrating a process for the production of a field emission cathode structure as one embodiment of this invention.

FIG. 2 is a partially sectioned perspective view illustrating a field emission cathode structure as one embodiment of this invention.

FIG. 3 is a cross section illustrating the essential part of a flat panel display device as one embodiment of this invention.

FIG. 4 is a perspective view illustrating the construction of the essential part of the flat panel display device shown in FIG. 3.

FIG. 5 is a perspective view illustrating the construction of the essential part of a flat panel display device as another embodiment of this invention.

FIG. 6 is a cross section illustrating the essential part of a flat panel display device as yet another embodiment of this invention.

FIGS. 7a, 7b, 7c and 7d are cross sections illustrating a process for the production of a flat panel display device as still another embodiment of this invention.

FIG. 8 is a diagram illustrating schematically the construction of an electron beam drawing device using a field emission cathode structure as one embodiment of this invention.

FIGS. 9a, 9b and 9c are cross sections illustrating a process for the production of a conventional field emission cathode structure.

FIG. 10 is a diagram to aid in explaining the construction of the conventional flat panel display device.

FIGS. 11a, 11b, 11c, 11d, 11e, 11f, 11g, and 11h are a series of model explanatory diagrams showing the second embodiment of the method for the production of a field emission cathode according to this invention.

FIGS. 12a, 12b, 12c, 12d, 12e, and 12f are a series of model explanatory diagrams showing the third embodiment of the method for the production of the field emission cathode according to this invention.

FIGS. 13a, 13b, 13c, 13d, 13e, and 13f are a series of model explanatory diagrams further showing the fourth embodiment of the method for the production of the field emission cathode according to this invention.

FIGS. 14a, 14b, 14c, 14d, 14e, and 14f are a series of model explanatory diagrams showing the fifth embodiment of the method for the production of the field emission cathode according to this invention.

## DESCRIPTION OF THE PREFERRED EMBODIMENTS

Now, this invention will be described below with reference to working examples of this invention illustrated in the annexed drawings.

Embodiment 1:

FIG. 1 is a diagram illustrating a process for the production of a field emission cathode structure as one embodiment of this invention. The method for producing the field emission cathode structure in this embodiment will be described below with reference to this diagram.

First, a hole of a pointed bottom is formed in a first substrate. As a method for forming the hole of this sort, the method which utilizes anisotropic etching of a Si single crystal substrate as shown below may be cited. First, a

thermally oxidized film of  $\text{SiO}_2$  approximately 0.1  $\mu\text{m}$  in thickness is formed by the technique of dry oxidation on a p-type Si single crystal substrate of a (100) crystal plane orientation and a resist is applied thereto by the technique of spin coating. Then, the resultant superposed layers are subjected to such patterning operations as exposure and development by the use of a stepper so as to form opening parts each of the square of 1  $\mu\text{m}$ . The  $\text{SiO}_2$  film is etched with a mixed  $\text{NH}_4\text{F}.\text{HF}$  solution. By performing the anisotropic etching with an aqueous 30 wt % KOH solution after the removal of the resist, the hole 12 of the shape of an inverted pyramid 12 is formed to a depth of 0.71  $\mu\text{m}$  in a Si single crystal substrate 11 as illustrated in FIG. 1a.

Then, the  $\text{SiO}_2$  film is provisionally removed by the use of a mixed  $\text{NH}_4\text{F}.\text{HF}$  solution and a thermally oxidized insulating layer 13 of  $\text{SiO}_2$  is superposed on the Si single crystal substrate 11 inclusive of the interior of the hole 12 as illustrated in FIG. 1b. In the present example, the thermally oxidized insulating layer 13 of  $\text{SiO}_2$  was formed in a thickness of 0.5  $\mu\text{m}$  by the technique of wet oxidation. Optionally, this insulating layer 13 may be formed by depositing  $\text{SiO}_2$  as by the technique of CVD. Since the thermally oxidized layer of  $\text{SiO}_2$  has a dense texture and allows easy control of the thickness thereof and also since the fact that the thermally oxidized layer is formed in a swelled state on the inner wall of the holes brings about an effect of imparting enhanced sharpness to the tips of the holes, the present working example adopted a thermally oxidized film for the insulating layer and selected the thickness of this thermally oxidized film in the range of from 0.03  $\mu\text{m}$  to 0.8  $\mu\text{m}$  in due consideration of the role to be performed by the insulating layer and on condition that the opening parts have a size of 1  $\mu\text{m}$ . of course, this thickness is subject to change depending on the size of the opening parts and the magnitude of voltage to be applied.

The thermally oxidized layer of  $\text{SiO}_2$  also functions as an etching stopper layer, in addition to the effect of enhanced sharpness to the tips of the emitter.

Subsequently, a W layer or a Mo layer, for example, is formed as an emitter material layer 14 on the aforementioned thermally oxidized layer 13 of  $\text{SiO}_2$ . The emitter material layer 14 is formed in such a manner that it will thoroughly fill up the holes 12 and, at the same time, permit continuity of the holes 12 to the other parts. In the present working example, the emitter material layer 14 was formed in a thickness of 2  $\mu\text{m}$  by the technique of sputtering. The emitter material layer of this invention is not always required to fulfill the part of a structural layer. Generally, therefore, the thickness of the emitter material layer 14 is approximately in the range from 0.1 to 5  $\mu\text{m}$  suffices. Further, an ITO conductive layer 15 is formed in a thickness of 1  $\mu\text{m}$ , for example, similarly by the technique of sputtering. Incidentally, this conductive layer 15 may be omitted, depending on the kind of substance of the emitter material layer 14. When this omission is effected, the emitter material layer 14 concurrently serves as a cathode electrode layer.

When, in this case, the emitter material layer 14 and the cathode electrode are formed of one same material, the field emission cathode structure to be obtained suffers from separation and deterioration only sparingly and enjoys ideal quality because they are enabled to share a continued texture.

In the meanwhile, a Pyrex glass substrate (1 mm thick) 17 having the rear surface thereof coated with an Al layer 16 of a thickness of 0.3  $\mu\text{m}$  is prepared as a structural substrate destined to form a second substrate and the glass substrate 17 and the Si single crystal substrate 11 mentioned above are

interjoined through the medium of the emitter material layer 14 as illustrated in FIG. 1c. For this junction, the technique of electrostatic bonding can be adopted. The electrostatic bonding technique is effected by applying an electric field of 50 to 500 V with the emitter side as the plus pole and the glass substrate side as the negative pole. This technique contributes to decreasing the weight and thickness of the cathode device to be produced.

The Al layer 16 on the rear surface of the glass substrate 17 is removed with a mixed acid solution of  $\text{HNO}_3\text{CH}_3\text{COOH}\text{HF}$  and then the Si single crystal substrate 11 alone is removed by etching with a mixed aqueous solution of ethylene diamine, pyrocatechol, and pyrazine (ethylene diamine:pyrocatechol:pyrazine:water= 75 cc:12 g:3 mg:10 cc). At this time, the thermally oxidized layer of  $\text{SiO}_2$  13 effects as an etching stopper layer, the thermally oxidized insulating layer 13 of  $\text{SiO}_2$  is exposed and, at the same time, pyramidal protrusions 18 of the emitter material covered by the thermally oxidized insulating layer 13 of  $\text{SiO}_2$  as the etching stopper are thrust out as illustrated in FIG. 1d. The pyramidal protrusions 18 correspond to the parts of the emitter material filling the interiors of the holes 12 in the Si single crystal substrate 11. Then, as a gate electrode layer 19, a W layer, for example, is formed on the thermally oxidized insulating layer 13 of  $\text{SiO}_2$  along the shapes of the protrusions 18 covered with the thermally oxidized insulating layer of  $\text{SiO}_2$  as illustrated in FIG. 1e. In the present working example, the W layer 19 was formed in a thickness of 0.5  $\mu\text{m}$  by the technique of sputtering. Further, a photoresist 20 is formed to such an extent that the tips of the protrusions 18 covered with the gate electrode layer 19 and the thermally oxidized insulating layer 13 of  $\text{SiO}_2$  may be slightly concealed. In the present working example, the photoresist 20 was applied in a thickness of about 0.9  $\mu\text{m}$  by the technique of spin coating.

In the above, when the gate electrode layer is formed, the thermally oxidized insulating layer of  $\text{SiO}_2$  13 which functions as the etching stopper layer is left as an insulator.

Though the insulating quality decreases, if it is necessary to provide the distance between the gate electrode 19 and the emitter more widely, the thermally oxidized insulating layer of  $\text{SiO}_2$  13 may be removed by etching with the mixed solution of  $\text{NH}_4\text{F}$  and HF, and a Si oxidized layer may be deposited by the CVD method or the electron beam vacuum depositing method to form a new  $\text{SiO}_2$  layer having a desired thickness, thereby the distance between the gate electrode 19 and the emitter being selected freely.

The photoresist 20 is removed by dry etching with oxygen plasma in such a manner that tips 19a of the gate electrode layer 19 (inclusive of the tips 13a of the thermally oxidized insulating layer 13 of  $\text{SiO}_2$ ) along the pyramidal protrusions 18 may be exposed to a depth of about 0.7  $\mu\text{m}$  as illustrated in FIG. 1f. Thereafter, the parts of the gate electrode layer 19 overlying the tips 18a of the pyramidal protrusions 18 are removed by reactive ion etching to open the parts of the gate electrode layer 19 corresponding to the tips of the pyramidal protrusions 18 as illustrated in FIG. 1g.

After the resist 20 is removed, the parts of the thermally oxidized insulating layer 13 of  $\text{SiO}_2$  encircling the tips 18a of the pyramidal protrusions 18 are selectively removed by etching with a mixed solution of  $\text{NH}_4\text{F}\text{HF}$ . As a result, opening parts 19b of the gate electrode layer 19 are formed and, at the same time, the tips 18a of the pyramidal protrusions 18 of the emitter material are exposed to give rise to pyramidal cathodes or emitters as illustrated in FIG. 1h.

The construction of the field emission cathode structure obtained by the working example of production described

above is illustrated in FIG. 2. Incidentally, FIG. 2 represents a case of omitting the formation of the ITO conductive layer 15. In the field emission cathode structure, the emitter material layer 14 concurrently serving as a cathode electrode layer is formed as held in direct contact on the glass substrate 17 serving as a structural substrate. On the emitter material layer 14, the pyramidal protrusions 18 are integrally formed as emitters (as W emitters, for example). The pyramidal emitters 18 correspond to the parts of the emitter material filling the interiors of the holes 12 formed in the Si single crystal substrate 11.

The pyramidal emitters 18 are covered with the thermally oxidized insulating layer 13 of  $\text{SiO}_2$  except for the tips 18a thereof which are destined to form electron discharge parts. The W layer destined to serve as the gate electrode layer 19 is formed through the medium of the thermally oxidized insulating layer 13 of  $\text{SiO}_2$ . The gate electrode layer 19 is formed along the shapes of the pyramidal emitters 18 and is provided with the opening parts 19b which are formed so as to encircle the tips 18a of the emitters 18. The tips 18a of the pyramidal emitters 18 are positioned inside the openings 19b of the gate electrode layer 19 and are adapted to discharge electrons by way of field emission through the medium of the opening parts 19b.

In the working example described above, since the thermally oxidized insulating layer 13 of  $\text{SiO}_2$  is formed first on the Si single crystal substrate 11 provided with the holes 12 and the emitter material layer 14 is subsequently formed by deposition, the field emission cathode structure consequently produced allows accurate control of the gaps between the gates and the emitters as compared with the conventional field emission cathode structure which has the insulating layer formed as by the technique of CVD. Generally, Si is used for the field emitters which by nature are subjected to anisotropic etching. The field emission cathode structure of this invention does not limit the material for emitters to Si. It instead allows use of various materials such as W which have a low work function. Since the pyramidal emitters 18 are formed by filling the holes 12 formed in the Si single crystal substrate 11 with the emitter material, the emitters 18 conforming to the shapes of the holes 12 can be produced with high repeatability. Since the holes 12 are enabled to assume the shape of an inverted pyramid having an ideally pointed bottom owing to the high repeatability of the shaping by anisotropic etching and the full growth of the thermally oxidized insulating layer 13 of  $\text{SiO}_2$  within the holes 12, the pyramidal emitters 18 to be produced are allowed infallibly to acquire sharply pointed tips 18a of an eminently uniform height.

The emitters 18 of this quality enjoy a generous improvement in efficiency of field emission and uniformity thereof and make a great contribution to improving the efficiency and uniformity of various electronic devices using the field emission cathode structure. Further, in the field emission cathode structure of this invention, since the thermally oxidized insulating layer 13 of  $\text{SiO}_2$  is formed along the pyramidal shapes of the emitters 18, the parts of the emitters other than the tips thereof serving to discharge electrons are electrically insulated. Thus, the concentration of electric fields to the tips is increased, the efficiency of field emission is enhanced, and the stability of the operation of field emission is improved.

Further, owing to the procedure which comprises forming the emitter material layer 14 inclusive of the pyramidal emitters 18 on the Si single crystal substrate (first substrate) 11, joining this layer 14 to the structural substrate (glass substrate) 17, and subsequently dissolving and remov-

ing the unnecessary Si single crystal, a multiplicity of Si single crystal substrates 11 having the pyramidal emitters 18 formed thereon can be integrated on one and the same structural substrate 17. Thus, the area for the formation of cathode parts can be easily enlarged and the formation of the field emission cathode structure of a large surface area can be accomplished. Since the unnecessary Si single crystal is dissolved and removed and, as a result, the emitter material layer 14 is made to assume the state of being directly (or through the medium of the conductor layer 15) superposed on the structural substrate 17, the produced field emission cathode structure does not suffer from an increase in thickness like the conventional cathode structure. Thus, cathode structures of a small thickness can be easily formed within a large area, indicating that the productivity of field emission cathode structures can be improved and the adaptability thereof to various electronic devices can be realized.

Moreover, the accurate control of the gaps between the gates and the emitters and the improvement of the reproducibility of the shapes of emitters 18 contribute to curbing the currents of electrons between the gates and the emitters. The emission of electrons, therefore, can be attained with high efficiency. In the flat panel display device, for example, the efficiency emission from the picture elements corresponding to the individual cathode parts can be heightened and, at the same time, the inconsistency of luminance among the picture elements can be curbed.

#### Embodiment 2:

The second embodiment of this invention will be described with reference to FIGS. 11a, b, c, d, e, f, g, and h.

First, a Si single crystal substrate (first supporting substrate) 11 is prepared. One main surface of this supporting substrate 11 is anisotropically etched to form a hole 12 (in the shape of an inverted pyramid) having a tip part pointed at a prescribed angle as shown in FIG. 11a.

To be more specific, a thermally oxidized film ( $\text{SiO}_2$  film) about 0.1  $\mu\text{m}$  in thickness is formed as by the dry oxidation method on the main surface of a p-type Si single crystal substrate 11 having a crystal face orientation of (100) and a resist is applied by the spin coating method to the surface of the thermally oxidized film.

Then, the resist is patterned so as to obtain an opening of the shape of the square of 0.8  $\mu\text{m}$ , for example, through the treatments of exposure and development with the aid of a stepper, the exposed area of the oxide film ( $\text{SiO}_2$  film) is selectively etched with a mixed solution of  $\text{NH}_4\text{F} \cdot \text{HF}$ , the resist is removed, and the anisotropic etching is carried out with an aqueous 30% KOH solution to give rise to the hole 12 of the shape of an inverted pyramid 0.56  $\mu\text{m}$  in depth on the main surface of the Si single crystal substrate 11.

Subsequently, the thermally oxidized film which has served as the mask is removed with the mixed solution of  $\text{NH}_4\text{F} \cdot \text{HF}$  and the Si layer 73 containing a P-type impurity at a concentration of not less than  $3 \times 10^{19} \text{ cm}^{-3}$  such as, for example, a B-diffused Si layer 73 having a thickness of 0.3  $\mu\text{m}$ , is superposed in a substantially uniform thickness on the surface of the Si single crystal substrate 11 containing the hole 12 of the shape of an inverted pyramid. The B-diffused Si layer 73 in this case functions as an etching stopper layer (sacrifice layer) during the removal of the Si single crystal substrate 11. This layer 73 can be used in its unmodified form as a gate electrode layer when the concentration of the p-type impurity is so high as to fall in the range of from  $10^{20}$  to  $10^{21} \text{ cm}^{-3}$  and the electric resistance is so low as to fall in the neighborhood of  $10^{-4} \Omega \cdot \text{cm}$ . In this case, the number of man-hours can be decreased and the distance between the gate and the emitter can be shortened to permit desirable mutual approximation.

Then, the Si single crystal substrate 11 provided with the p-type impurity diffusion Si layer 73 is subjected to a treatment of thermal oxidation to effect thermal oxidation of the surface of the p-type impurity diffusion Si layer 73 and give rise to the insulator layer 13 having a thickness of 0.2  $\mu\text{m}$ .

After the insulator layer 13 has been formed as described above on the surface of the p-type impurity diffusion Si layer, an emitter material such as, for example, W, Mo, or Ta is sputtered on the surface of the insulator layer 13 so as to fill the pyramidal hole covering the p-type impurity diffusion Si layer 73 and the insulator layer 13, form the emitter projection 18 conforming to the hole mentioned above, and also form the emitter material layer 14 having a smoothly finished surface and a thickness of about 0.8  $\mu\text{m}$ .

Further on the surface of the emitter material layer 14, an electroconductive layer 15 such as, for example, an ITO (indium-tin type oxide) layer 15 having a thickness of about 1  $\mu\text{m}$ , is superposed as by sputtering to produce such a laminate as shown in FIG. 11b. Here, the ITO layer 15 may be omitted, depending on the material used for the emitter material layer 14. When this omission is made, the emitter material layer 14 goes to play the part of a cathode electrode layer concurrently.

The second supporting substrate (structural substrate) such as, for example, a Pyrex glass sheet 17 having the rear surface (back surface) thereof coated with an Al layer 16 destined to serve as an electrostatic bonding electrode and having a thickness of about 0.4  $\mu\text{m}$  is superposed on the laminate mentioned above. The ITO layer 15 and the Al layer 16 are interjoined by the so-called electrostatic bonding method which resides in applying a voltage of the order of some hundreds of V between the layers (FIG. 11c). Though this union of the two layers may be accomplished by the use of an adhesive agent, the electrostatic bonding method proves more advantageous from the viewpoint of providing the produced field emission cathode with greater reduction in weight and thickness.

After the Pyrex glass sheet 17 as the structural substrate has been joined to the laminate, the rear coat (Al) layer 16 of the Pyrex glass sheet 17 is removed by etching as with a mixed acid solution of  $\text{HNO}_3 \cdot \text{CH}_3\text{COOH} \cdot \text{HF}$ , for example.

Then, the Si single crystal substrate 11 as the first supporting substrate is removed by etching by the use of an aqueous solution containing the mixture of ethylene diamine, pyrocatechol, and pyrazine (mixing ratio 75 cc:12 g:3 mg:10 cc) to give rise to a laminate composed of the insulator layer 13 and the emitter layer 14 provided with the pyramidal projection 18 (conforming to the aforementioned pyramidal hole 12) and covered by the p-type impurity diffusion Si layer 73 as shown in FIG. 11d. During this process of etching, the p-type impurity diffusion Si layer 73 functions as an etching stopper layer for the Si single crystal substrate 11 and discharges the role of protecting the insulator layer 13 having a small film thickness and the pyramidal projection 18 of the main body of the emitter having a sharp pointed tip against corrosion by the etching solution mentioned above.

Then, on the surface of the p-type impurity diffusion Si layer 73 which has been exposed by the removal by etching of the Si single crystal substrate 11, W is deposited in the form of a coat in a thickness of about 0.5  $\mu\text{m}$  as by the sputtering method, for example. To the surface of the W coat layer 19 formed as described above, a photoresist layer 20 is applied as by the spin coating method in a thickness such as, for example, about 0.9  $\mu\text{m}$  which is enough to conceal a tip part 19t of the projection on the surface of the W coat

layer 19 embracing therein the pyramidal projection 18 of the emitter as shown in FIG. 11e.

Thereafter, by the dry etching treatment using oxygen plasma, part of the photoresist layer 20 is removed so that the tip part 19t of the projection of the W coat layer containing the projection 18 of the emitter may be exposed in a thickness of about 0.7  $\mu\text{m}$  through the surface as shown in FIG. 11f.

Subsequently, by the reactive ion etching treatment, the tip part 19t of the projection of the W coat layer 19 which has been exposed by the removal by etching of part of the photoresist layer 20 is selectively removed to form the gate electrode layer 19a provided with an opening 19b exposing the tip part of the projection covering the impurity diffusion layer 73 and the insulator layer 13 as shown in FIG. 11g.

The remainder part of the photoresist layer 20, namely the part which has functioned as a mask for the selective etching of the tip part 19t of the W coat layer, is subsequently removed. Then, the impurity diffusion layer 73 and the insulator layer 13 covering the tip part 18t of the projection 18 of the emitter are selectively removed by etching with the mixed solution of  $\text{NH}_4\text{F}\text{HF}$  so as to expose the tip part 18t of the projection 18 of the emitter 18.

As a result, the field emission cathode is obtained which is so constructed as to expose the tip part 18t of the pyramidal projection 18 of the main body of the emitter through the opening 19b of the gate electrode layer 19a as shown in FIG. 11h.

In accordance with the method of production described above, the high-concentration impurity diffusion layer 73 doped with an impurity is formed on the surface of the supporting substrate 11 provided with the hole formed by anisotropic etching and pointed sharply in the tip (bottom surface side) thereof, the insulator layer 13 is further formed thereon by the thermal oxidizing method, and subsequently the emitter material layer 14 is formed in such a manner as to fill the hole mentioned above. During the course of this process, the hole having a sharply pointed tip is formed in a prescribed shape with high repeatability by the anisotropic etching. Further, since the formation of the insulator layer 13 by the thermal oxidation permits growth of  $\text{SiO}_2$  of high density and since the high-concentration impurity diffusion layer 73 provides effective protection of the insulator layer 13 and the emitter material layer 14 against corrosion by etching, the emitter function part is formed which possesses a sharp pointed tip part uniform in height and shape and also excels in uniformity of quality.

Thus, the provision of field emission cathodes with stabilized quality can be realized. Further, since the insulator layer 13 can be formed in a fully accurately controlled thickness by the thermal oxidizing method, the distance between the emitter function part mentioned above and the gate electrode layer 19a (emitter-gate distance) is controlled with high accuracy. Thus, the field emission cathode is capable of operating at a relatively low voltage to effect highly efficient emission.

The embodiment described above represents a case of having the gate electrode layer 19a superposed on the surface of the impurity diffusion layer 73. The operation and effect of the embodiment under consideration are similarly attained by causing the impurity diffusion layer 73 to function as a gate electrode layer when this impurity diffusion layer 73 has a high impurity concentration and a high electric resistance or by removing the impurity diffusion layer 73 participating mainly in the selective etching of the supporting substrate 11 thereby exposing the insulator layer 13 and superposing the gate electrode layer 19a on the surface of the exposed insulator layer 13.

The effect manifested by the embodiment is invariable when the impurity mentioned above is a p-type B, Al, Ga, or In, an n-type P, As, or Ti, or an i-type Ge or Sn.

It is allowed in this invention to use as the material for the first supporting substrate such substance as GaAs in the place of Si single crystal and as the emitter material Mo, Ta, Si, or other substance having a low work function in the place of W.

The operation and effect of the present embodiment are obtained invariably when a soda glass plate is used in the place of the Pyrex glass plate as the second supporting substrate (structural substrate).

Further, the embodiment described above represents a case of handing the field emission cathode as a unitary article. As a matter of course, a group of such field emission cathodes may be arrayed in the form of a matrix, for example, on one Si single crystal sheet to produce a planar field emission cathode.

As described above, the field emission cathode of the first embodiment of this invention has originated in the interest drawn to the fact that a pyramidal or conical hole having a pointed tip can be formed on the surface of a supporting substrate by utilizing the anisotropy of etching, the fact that a region converted into an impurity diffusion layer functions as an etching stopper layer, the fact that the impurity diffusion layer functions concurrently as a gate electrode layer when it has low resistance, and the fact that an acute oxide layer (insulator layer) is formed in a highly accurately controlled shape along a prescribed surface by the use of the thermal oxidation method. The field emission cathode of the present invention always enjoys excellent qualities of constantly displaying ideal uniformity of field emission, providing an effective operation at a low voltage, and obtaining high field emission efficiency.

Further, in accordance with the method for the production of the field emission cathode of the present invention, the field emission cathode which is endowed with such functional characteristics as mentioned above and is easily adapted for high integration can be manufactured with highly satisfactory yield and productivity (ability of quantity production). Thus, the method of production contemplated by this invention may well be rated as contributing greatly to the utilization of field emission cathodes of this type in practical applications.

#### Embodiment 3:

Figs. 12a, b, c, d, e, and f are a series of diagrams showing a process for the production of a field emission cathode as the third embodiment of this invention. The method of production according to the third embodiment will be described below with reference to these diagrams. In these diagrams, like parts found in the second embodiment are denoted by like reference numerals.

First, as shown in FIG. 12a, the Si single crystal substrate 11 offering low resistance and having a crystal face orientation of (100) is prepared as a first supporting substrate.

Then, the hole 12 sharply pointed toward the bottom part thereof is incised on one flat surface of the Si single crystal substrate 11 (hereinafter referred to as the first main surface) as shown in FIG. 12b. For the incision of the hole 12 of such a shape as described above, the method which utilizes the anisotropic etching of Si to be described hereinbelow may be adopted. To be specific, on the first main surface of the Si single crystal substrate 11 made of a Si single crystal having a crystal face orientation of (100), a thermally oxidized film of  $\text{SiO}_2$  is superposed in a thickness of about 0.1  $\mu\text{m}$  by the dry oxidizing method. Then, the photoresist is patterned so as to obtain an opening of the shape of the

square of 1  $\mu\text{m}$ , for example, through the treatments of exposure and development with the aid of a stepper and the thermally oxidized  $\text{SiO}_2$  film is etched by the use of the mixed solution of  $\text{NH}_4\text{F}.\text{HF}$  as an etchant. The photoresist is removed and the first main surface of the Si single crystal substrate 11 is subjected to the anisotropic etching by the use of an aqueous 30 wt % KOH solution as an etchant. As a result, the hole 12 of the shape of an inverted pyramid 0.71  $\mu\text{m}$  in depth is incised on the first main surface side of the Si single crystal substrate 11. Then, the thermally oxidized  $\text{SiO}_2$  film remaining on the surface of the Si single crystal substrate 11 is removed by the use of the mixed solution of  $\text{NH}_4\text{F}.\text{HF}$ , for example.

Subsequently, the thermally oxidized layer 13 is formed as shown in FIG. 3C on the first main surface of the Si single crystal substrate 11 including the inner wall surfaces of the hole 12 by subjecting the surfaces mentioned above to a treatment of thermal oxidation. In the present embodiment, the thermally oxidized layer 13 is formed by the wet method of thermal oxidation so as to acquire a thickness of 0.5  $\mu\text{m}$ . Then, on this thermally oxidized layer 13, the emitter material layer 14 using W or Mo is formed. This emitter material layer 14 is so formed as to cover the upper surface of the thermally oxidized layer 13 while filling the hole 12. In the present embodiment, the emitter material layer 14 is deposited by the sputtering method so as to form a film 2  $\mu\text{m}$  in thickness on the thermally oxidized layer 13 excepting the hole 12.

Then, as a second supporting substrate, the glass substrate 17 made of such a highly heat-resistant material as Pyrex glass and provided on the rear surface thereof with the Al layer 16 of a thickness of 0.3  $\mu\text{m}$  as a coating as shown in FIG. 12d is prepared. This glass substrate 17 is superposed on and joined fast to the surface of the emitter material layer 14 opposite to the surface thereof on which the projection 18 of a sharp pointed tip. For this union, the electrostatic bonding method may be adopted, for example. Then, the Al layer 16 on the rear surface of the glass substrate 17 is removed with the mixed acid solution of  $\text{HNO}_3.\text{CH}_3\text{OOH}.\text{HF}$ .

Then, the substrate in its entirety is inverted (upside down) so that the second main surface of the Si single crystal substrate 11 opposite to the first main surface thereof may fall on the upper side and the second main surface side of the Si single crystal substrate 11 opposite to the first main surface is removed by etching by the use of the so-called EDP, i.e. a mixed aqueous solution of ethylene diamine, pyrocatechol, and pyrazine (the ratio of ethylene diamine:pyrocatechol:pyrazine:water= 75 ml:12 g:0.45 g:10 ml in the present embodiment), as an etchant. In this case, the etching time is so controlled that the Si single crystal layer 11 may remain in a thickness allowing the tip part of the projection 18 of the emitter material layer 14 to be finally exposed and, at the same time, the lower part of the emitter material layer 14 to be coated with the Si single crystal layer 11 through the thermally oxidized layer 13 as shown in FIG. 12e. Thus, the Si single crystal substrate 11 is not wholly etched evenly in the direction of thickness thereof. The Si single crystal layer 11 is used as a gate electrode. Thus, the thermally oxidized layer 13 covering the sharply pointed tip part of the projection 18 of the emitter material layer 14 is exposed from the Si single crystal layer 11.

Now, the part of the thermally oxidized layer 13 which covers the tip part of the projection 18 of the emitter material layer 14 is removed by etching with the mixed solution of  $\text{NH}_4\text{F}.\text{HF}$  as an etchant to expose the sharp pointed tip part of the projection 18 partly from the Si single crystal layer 11 as shown in FIG. 12f. Thus, the emitter is obtained.

The method of production described above has the effect of enabling the field emission cathode contemplated by this invention to be formed with ease in addition to the effect manifested by the method of production of the second embodiment.

Embodiment 4:

FIGS. 13a, b, c, d, e, and f are a series of diagrams showing a process for the production of the field emission cathode of the fourth embodiment of this invention. The method production of the fourth embodiment will be explained below with reference to these diagrams. In these diagrams, like parts found in the second and the third embodiment are denoted by like reference numerals.

The present embodiment is characterized by superposing the etching stopper layer 73 having boron (B) diffused therein at a high concentration and having a small thickness on the Si single crystal substrate 11 and causing the advance of the etching of the Si single crystal substrate 11 from the second main surface side thereof to be stopped by this etching stopper layer 73. It, therefore, finds no use for such complicate control of the etching time as is encountered in the third embodiment and facilitates the formation of the field emission cathode of this invention to a greater extent.

First, the etching stopper layer 73 of a small thickness is formed on the first main surface of the Si single crystal substrate 11 having a crystal face orientation of (100) by diffusing on the surface mentioned above the ions of such an impurity as boron (B) at a high concentration of not less than  $10^{19} \text{ cm}^{-3}$ , for example. This high-concentration impurity diffusion is effected by the thermal diffusion method or the ion injection method, for example.

Then, as shown in FIG. 13b, the hole 12 pointed sharply toward the bottom part thereof is incised in the Si single crystal substrate 11 from the etching stopper layer 73 (first main surface) side in the same manner as in the second embodiment. For the incision of this hole 12, the method which resorts to the anisotropic etching of Si may be adopted similarly to the third embodiment. To be specific, the treatment of thermal oxidation by the dry method is performed on the surface of the etching stopper layer 73 to form a thermally oxidized  $\text{SiO}_2$  film in the etching stopper layer 73 to a depth of about 0.1  $\mu\text{m}$ . The photoresist (not shown) is further applied to the thermally oxidized  $\text{SiO}_2$  film by the spin coating method. Then, the photoresist is patterned as by the treatments of exposure and development by the use of a stepper, for example, so as to obtain an opening in the shape of the square of 1  $\mu\text{m}$ . The thermally oxidized  $\text{SiO}_2$  film is subsequently patterned by the use of the mixed solution of  $\text{NH}_4\text{F}.\text{HF}$  as an etchant. Then, the photoresist mentioned above is removed and the anisotropic etching is carried out with the pattern of the thermally oxidized  $\text{SiO}_2$  film as an etching mask and the aqueous 30 st % KOH solution as an etchant. Thus, in the etching stopper layer 73, the hole 12 having the shape of an inverted pyramid is incised in a depth of 0.71  $\mu\text{m}$  reaching beyond the first main surface of the Si single crystal substrate 11. Then, the thermally oxidized  $\text{SiO}_2$  film remaining on the surface of the etching stopper layer 73 is removed by the use of the mixed solution of  $\text{NH}_4\text{F}.\text{HF}$ , for example.

Here, an ideal etching speed is obtained even when the etching stopper layer 73 is formed on the Si single crystal substrate 11 because the aqueous KOH solution manifests a practically equal etching rate on the etching stopper layer 73 having boron (B) diffused at a high concentration therein and the Si single crystal. Even when the etching stopper layer 73 is formed on the Si single crystal substrate 11 as in the present embodiment, therefore, the hole 12 can be ideally

incised. Naturally, some other etchant may be used herein on the condition that it should be capable of etching the etching stopper layer 73.

Then, the treatment of thermal oxidation is performed on the wall surfaces of the etching stopper layer 73 and the Si single crystal substrate 11 which are exposed through the hole 12 and on the flat surface of the etching stopper layer 73 to form the thermally oxidized layer 13. During the course of the thermal oxidation, the etching stopper layer 73 gains in thickness. The thickness of the etching stopper layer 73 is set preparatorily during the formation of the Si single crystal substrate 11 so that the part of the thermally oxidized layer 13 covering the tip part of the pyramidal projection 18 may protrude from the etching stopper layer 73 even after the etching stopper layer 73 is inflated as described above. Then, in the same manner as in the third embodiment described above, such a material as W or Mo which makes an ideal emitter material is deposited on the thermally oxidized layer 13 to give rise to the emitter material layer 14.

Now, similarly to the third embodiment, the glass substrate 17 made of such a highly heat-resistant material as Pyrex glass and provided on the rear surface thereof with the Al layer 16 having a thickness of 0.3  $\mu\text{m}$  as a coating is prepared as shown in FIG. 13d. This glass substrate 17 is superposed on and attached fast to the surface of the emitter material layer 14 opposite to the surface thereof on which the pyramidal hole 18 pointed toward the tip thereof is formed. For this union, the electrostatic bonding method may be adopted similarly to the third embodiment. Then, the Al layer 16 on the rear surface of the glass substrate 17 is removed with the mixed acid solution of  $\text{HNO}_3\text{--CH}_3\text{OOH--HF}$ .

Then, as shown in FIG. 13e, the Si single crystal substrate 11 is removed by etching from the second main surface side opposite to the first main surface by the use of the so-called EDP, i.e. a mixed aqueous solution of ethylene diamine, pyrocatechol, and pyrazine (the ratio of ethylene diamine:pyrocatechol:pyrazine:water= 75 ml:12 g:0.45 g:10 ml in the present embodiment), as an etchant.

Here, since the etching stopper layer 73 is formed of a Si material having boron (B) diffused at a high concentration, the etchant like EDP which is used in the second embodiment manifests a considerably lower etching rate on the etching stopper layer 73 than on the single crystal of Si. As a result, the etching advancing in the Si single crystal substrate 11 from the second main surface side thereof is stopped by the etching stopper layer 73, with the result that the etching stopper layer 73 will remain practically intact. Thus, the thermally oxidized layer 13 covering the sharp pointed tip part of the projection 18 of the emitter material layer 14 can be partly exposed from the etching stopper layer 73.

Then, as shown in FIG. 13f, the part of the thermally oxidized layer 13 covering the tip part of the projection 18 of the emitter material layer 14 is removed by etching with the mixed solution of  $\text{NH}_4\text{F--HF}$  as an etchant to obtain partial exposure of the sharp pointed tip part of the projection 18 through the etching stopper layer 73. Thus, the emitter is obtained.

Incidentally, since the etching stopper layer 73 is formed of a Si material having boron (B) diffused therein at a high concentration and consequently enjoys high electric conductivity, it may be left in its unmodified form and used as a gate electrode.

The method of production of the fourth embodiment described above obviates the necessity of ensuring complicated control of the etching depth during the etching of the Si

single crystal substrate 11 from the second main surface side thereof as involved in the third embodiment. It, therefore, brings about the effect of enabling the field emission cathode to be formed with further increased ease in addition to the effects obtained by the methods of production of the second and the third embodiment.

Embodiment 5:

FIGS. 14a, b, c, d, e, and f are a series of diagrams showing a process for the production of the field emission cathode of the fifth embodiment of this invention. The method of production of the fifth embodiment will be explained with reference to these diagrams. In these diagrams, like parts found in the second and the third embodiment are denoted by like reference numerals. This fifth embodiment will be described below with emphasis centering on the characteristic parts thereof which differentiate this embodiment from the embodiments described above.

The method of production of the present embodiment is characterized by using an etching stopper layer 73a formed of an n-type Si material in the place of the etching stopper layer 73 of the third embodiment described above and causing the etching advancing in the Si single crystal substrate 11 from the second main surface to be stopped by applying a reverse voltage to the etching stopper layer 73a.

First, as shown in FIG. 14a, the Si layer 73a is formed in a small thickness as by the thermal diffusion method or the ion injection method on the Si single crystal substrate 11 made of a p-type Si single crystal having a crystal face orientation of (100) and the Si single crystal substrate 11 and the Si layer 73a are joined by the pn junction across the interface.

The subsequent steps shown in FIGS. 14b through 14d are practically the same as the corresponding steps used in the fourth embodiment described above.

The present embodiment is then characterized by adopting the electrochemical etching method at the step of removing the Si single crystal substrate 11 shown in FIG. 14e.

This method resides in applying reverse voltage to the pn junction produced in the interface between the etching stopper layer 73a and the Si single crystal substrate 11 in an aqueous KOH solution, for example, thereby selectively etching the p-type Si single crystal substrate 11 exclusively and allowing the n-type Si layer 73a to remain intact in spite of the etching.

Thus, the Si single crystal substrate 11 is progressively etched from the second main surface side thereof until the Si single crystal substrate 11 is corroded out practically throughout the entire thickness thereof and only the tip part of the projection 18 of the emitter material layer 14 is exposed through the etching stopper layer 73a.

The steps which follow are identical to the corresponding steps involved in the embodiments described above. Specifically, the part of the thermally oxidized layer 13 covering the tip part of the projection 18 of the emitter material layer 14 is removed by etching with the mixed solution of  $\text{NH}_4\text{F--HF}$  as an etchant as shown in FIG. 14f. Thus, the sharp pointed tip part of the projection 18 is partly exposed through the Si single crystal layer 73a. The emitter is obtained as a result.

Similarly to the embodiments described above, the fifth embodiment under consideration offers the method of production which enables the gap between the emitter and the gate electrode to be formed accurately and easily.

In the fourth and the fifth embodiment described thus far, the etching stopper layer 12 having boron (B) diffused therein at a high concentration or the n-type Si layer 73a may be preparatorily formed by epitaxial growth on the first

main surface of the Si single crystal substrate 11 at the step of FIG. 13a or FIG. 14a.

Naturally, the materials for the component layers, the formation of the layers in the form of film, the method of patterning, and the like may be variously altered without departing from the spirit of the present invention.

As clearly described in detail above, this invention has been perfected for the purpose of realizing the fact that a pyramidal or conical hole pointed toward the tip thereof can be formed in a supporting substrate by utilizing the anisotropy of etching, the fact that a region converted into an impurity diffusion layer functions as an etching stopper layer, the fact that this impurity diffusion layer functions concurrently as a gate electrode layer depending on the magnitude of resistance thereof, and the fact that an acute oxide layer (insulator layer) can be formed accurately along prescribed surfaces by utilizing the thermal oxidation method.

The field emission cathode according to this invention is endowed with excellent qualities of constantly manifesting ideal field emission uniformly, operating effectively even at a low voltage, and obtaining high efficiency in field emission. Then, the method of this invention for the production of a field emission cathode allows field emission cathodes which are furnished with such functional characteristics as mentioned above and are readily adapted for further integration to be manufactured in a highly satisfactory yield with an ability of quantity production (mass production).

Now, the flat panel display device using the field emission cathode structures obtained by the aforementioned working example will be described specifically below.

In the flat panel display device 30 of the present working example, the glass substrate 17 having a multiplicity of field emission pyramidal emitters 18 formed thereon (hereinafter referred to as "cathode plate 21") and a glass face plate 33 having a phosphor layer 31 and a transparent electrode (anode electrode) layer 32 made of ITO sequentially superposed thereon are opposed across a prescribed gap to each other as illustrated in FIG. 3 and they jointly form a vacuum housing. Thus, the cathode plate 21 is used as part of the vacuum housing.

On the cathode plate 21, the emitter material layers 14 concurrently serving as cathode electrodes and gate electrode layers 19 are arranged after the fashion of a mutually intersecting network as illustrated in FIG. 4 and cathode forming regions 22 destined to form individual picture elements are set in place one each at the points of intersection of the network. The cathode forming regions 22 corresponding one each to the picture elements are severally provided with a multiplicity (50, for example) of pyramidal emitters 18. The phosphor layers 31 formed on the glass face plate 33 are each composed of a red emission phosphor layer 31a, a green emission phosphor layer 31b, and a blue emission phosphor layer 31c which correspond to each picture element. These phosphor layers are disposed correspondingly to the cathode forming regions 22. The phosphor layers 31a, 31b, and 31c are arranged as sequentially repeated in the horizontal direction.

When the flat panel display device 30 constructed as described above is operated by applying a voltage of 30 V between the gates and the cathodes and a voltage of 200 V between the anodes and the cathodes in accordance with a picture element signal, it produces an image of fine quality which excels in the luminance of light from the picture elements and suffers from inconsistency of the luminance among the picture elements only sparingly.

In the flat panel display device of this working example, images excelling in luminance of emitted light and suffering

only sparingly from inconsistency of luminance of the emitted light can be infallibly produced because the pyramidal field emitters 18 used in the device excel in accuracy of shaping and uniformity of shape and, at the same time, enjoy outstanding accuracy of the control of the gaps between the gates and the emitters. Further, since the field emission cathodes used in the device excel in the efficiency of emission of electrons, they make a contribution to a decrease in the power consumption by the device.

10 The cathode plate 21 which forms part of the vacuum housing has the glass substrate (structural substrate) 17 as its base and, therefore, possesses strength enough to withstand a high degree of vacuum. Further, when a multiplicity of Si single crystal substrates (11) having emitters 18 formed in advance thereon are deposited fast on the glass substrate 17 during the manufacture of cathodes, the flat panel display device can be easily produced as furnished with a large image screen. Even in this case, the glass substrate can maintain sufficient strength.

20 Now, the flat panel display device produced in another working example of this invention will be described below with reference to FIG. 5.

25 In the flat panel display device 40 of this working example, a red emission phosphor layer 41a, a green emission phosphor layer 41b, and a blue emission phosphor layer 41c are severally formed as second phosphor layers on the gate electrode layer 19 corresponding to a relevant cathode forming region 22. These phosphor layers 41a, 41b, and 41c on the gate electrode layer 19 side are respectively identical 30 in color to the opposed phosphor layers 31a, 31b, and 31c on the glass face plate 33 side. The phosphor layers 41a, 41b, and 41c on the gate electrode layer 19 side may be formed by the technique of spattering, for example. When the size of each picture element is large, they may be formed by the printing technique. The construction of the flat panel display device 40 except for what has been described above is presumed to be identical to that of the flat panel display device 30 described above.

35 When the flat panel display device 40 constructed as described above is operated by applying a voltage of 30 V between the gates and the cathodes and a voltage of 200 V between the anodes and the cathodes in accordance with a picture element signal, it produces an image of ideal quality which further excels in luminance of emission of light from the picture elements and suffers only sparingly from inconsistency of luminance among the picture elements.

40 In the conventional field emission cathode structure, the discharge current (electron current) between the cathodes and the anodes is approximately 50% to 80% of the discharge current obtained in the conventional C-CRT, with most of the remainder of the current flowing between the gates and the cathodes. When the phosphor layers 41a, 41b, and 41c are formed in advance also on the gate electrode layer 19 as in the flat panel display device 40 of the present working example, these layers emit light efficiently and the light is reflected by the gate electrode layer 19 itself which is made of a metallic material. Thus, the gate electrode layer 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 952

methods of manufacture can be effectively utilized for the fabrication of the device in question. Particularly when the conventional cathodes produced by the technique of rotary vacuum deposition illustrated in FIG. 9 which are considered to generate large currents of emission between the gates and the cathodes are adopted, the second phosphor layers on the gate electrode layer manifest their effect more conspicuously.

When the emitter 7 formed by the technique of rotary oblique vacuum deposition in the pinhole 5 dug in the insulating layer 2 of  $\text{SiO}_2$  superposed on the Si single crystal substrate 1 as illustrated in FIG. 6 is used, the second phosphor layer 41 is disposed on the gate electrode layer encircling the pinhole 5. By the use of this construction, the favorable efficiency of emission can be obtained and the inconsistency of luminance among the picture elements can be curbed even when there is used the emitter 7 produced by the technique of rotary oblique vacuum deposition which entails heavy inconsistency in the distances between the gates and the emitters and in the shapes of emitters and tends to enlarge the currents of emission between the gates and the cathodes.

Now, the procedure for the production of the field emission cathodes for use in the flat panel display device contemplated in yet another working example of this invention which has phosphor layers formed also in the opening parts of emitters in the gate electrode layer will be described below with reference to FIG. 7.

First, an insulating layer 52 of  $\text{SiO}_2$  1.2  $\mu\text{m}$  in thickness is formed by the technique of CVD on a Si substrate 51. Then, a Mo layer 53 0.5  $\mu\text{m}$  in thickness is formed by the technique of electron beam vacuum deposition on the insulating layer 52 of  $\text{SiO}_2$ . A resist is applied to the Mo layer 53 by the technique of spin coating and subjected to patterning by exposure to an electron beam. After the resist is removed, the Mo layer 53 is selectively etched to form an opening part 54. After the resist is completely removed, the insulating layer 52 of  $\text{SiO}_2$  is etched with a HF solution to form a hole 55 in the insulating layer 52 of  $\text{SiO}_2$ . Then, the Si substrate 51 is rotated parallelly to the surface of the substrate and Al is obliquely vacuum deposited as a separating layer on the Mo layer 53 to give rise to an Al layer 56. The process described thus far is depicted in FIG. 7a.

Then, the Si substrate 51 is rotated parallelly to the surface of the substrate and, at the same time, Mo is deposited on the Si substrate 51 perpendicularly thereto by the technique of electron beam vacuum deposition. Since a Mo layer 57 is deposited not only on the Al layer 56 and the Si substrate 51 but also on the lateral surfaces of the Al layer 56, the diameter of the opening part 54 gradually decreases. Since the range of vacuum deposition of Mo on the Si substrate 51 inside a hole 55 continues to decrease in consequence of the decrease of the diameter, a conical emitter 58 of Mo is formed on the Si substrate 51. The process thus far described is depicted in FIG. 7b.

After the Mo layer 57 and the Al layer 56 are moved [FIG. 7c], the Si substrate 51 is rotated parallelly to the surface of the substrate and, at the same time, red, green, and blue phosphor layers 59 are deposited in an oblique direction such as, for example, at an angle of 75 degrees relative to the axis of rotation by the technique of oblique vacuum deposition or oblique spattering to give rise to the opening part 54. Thus the cathode of the present working example is completed. The process thus far described is illustrated in FIG. 7d.

The flat panel display device using the cathode plate which is obtained as described above allows the currents of

electrons between the gates and the cathodes to be injected efficiently into the phosphor layers 59 as compared with the flat panel display device of the preceding working examples having the phosphor layers formed only on the gate electrode layer because the phosphor layers are formed additionally in the opening parts 54 of the gate electrode layer (Mo layer 53). When this flat panel display device is operated by applying a voltage of 30 V between the gates and the cathodes and a voltage of 200 V between the anodes and the cathodes, therefore, it produces an image of still better quality enjoying high luminance of the picture elements and suffering only sparingly from inconsistency of luminance.

Now, as another working example of the electron device of this invention, an electron beam drawing device will be described below with reference to FIG. 8.

FIG. 8 is a schematic diagram of the electron beam drawing device using the field emission cathode structures manufactured as described in the preceding working example. In the diagram, 61 stands for a field emission cathode provided with pyramidal emitters and manufactured as described in the preceding working example, 62 for a Si wafer, 63 for a stage, and 64 for a shock-absorbing base. The electron beam e radiated from the field emission cathode 61 into the interior of a container 65 which is maintained at a high degree of vacuum (about  $7 \times 10^{-8}$  Torr) is modulated (on/off control) in accordance with a signal of picture information by means of an electron source drive device 66 and also deflected in accordance with the signal of drawing information by a deflecting electrode 67 in the same manner as with the electron source drive device 66 to draw a pattern on the Si wafer 62. In the present working example, for the purpose of improving the convergence of the electron beam e emitted as described above, a converging electromagnetic lens 68 is installed and is controlled with an electromagnetic lens drive device 69. The stage 63 and the deflecting electrode 67 are synchronized by means of a synchronizing control mechanism 70.

In the electron beam drawing device constructed as described above, a fine pattern is drawn on the Si wafer 62 by applying a voltage of 30 V to the field emission cathode 61 thereby effecting emission of electron beam e and, at the same time, carrying out the deflection of the electron beam e and the motion of the stage 63 in accordance with the signal of drawing information.

The preceding working examples represent cases of using the field emission cathode structures of this invention in the flat panel display device and the electron beam drawing device. These are not the only devices that allow practical application of the field emission cathode structures of this invention. Other various electronic devices such as, for example, ultraspeed microwave devices, power devices, and electron beam devices equally allow effective use of the field emission cathode structures of this invention.

As described above, the method for the production of the field emission cathode structure contemplated by this invention allows stable production of emitters excelling in reproducibility of shape and uniformity (sharpness of tips, for example) and permits accurate control of gaps between the gates and the emitters. Thus, field emission cathode structures of high quality enjoying excellent efficiency of field emission and thoroughly curbing the inconsistency of the efficiency can be manufactured with high reproducibility. Since the cathode structures are allowed to utilize enlarged regions for the formation of their own without entailing an increase in thickness, they lend themselves to enhancing the productivity of the operation embodying the invention and,

at the same time, realizing effective adaptation for various electronic devices. Further, the field emission cathode structure of this invention manifests ample strength when it is used as part of the housing of a device and, therefore, can be used suitably in the flat panel display device, for example. The present invention enhances the luminance of the light emitted from the picture elements and curbs the inconsistency of the luminance among the individual picture elements.

What is claimed is:

1. A method for the production of a field emission cathode structure, comprising the steps of:

providing a first substrate with holes of a sharp point; forming an insulating layer on the surface of said first substrate inclusive of the surface of said holes;

forming an emitter material layer on said insulating layer and, at the same time, filling the interiors of said holes with said emitter material;

joining said first substrate covered with said emitter material layer to a second substrate made of a structural substrate through the medium of said emitter material layer, removing said first substrate by etching from said joined substrates so as to expose said insulating layer thereby allowing protrusions made of said emitter material filling the interiors of said holes and possessing said insulating layer as a surface layer thereof to thrust out;

forming a gate electrode layer on said insulating layer inclusive of said protrusions; and

removing part of said insulating layer and said gate electrode layer at the tips of said protrusions thereby giving birth to emitters possessing an exposed tip.

2. A method according to claim 1, wherein said insulating layer is obtained by thermally oxidizing the surface of said first substrate.

3. A method according to claim 1, wherein a conductive layer is formed on said emitter material layer.

4. A method according to claim 1, wherein said union of said first substrate and said second substrate is attained by the technique of electrostatic bonding.

5. A method for the production of a field emission cathode structure, comprising the steps of:

preparing a first substrate made of a single crystal material;

selectively etching said first substrate thereby forming on the surface of said substrate at least one hole having a sharp point;

forming an oxide layer on the surface of said first substrate provided with said at least one hole;

forming an emitter material layer in a uniform thickness on said oxide layer and, at the same time, filling said at least one hole with said emitter material;

preparing a second structural substrate made of a glass material;

joining said first substrate provided on the surface thereof with said emitter material layer to said second structural substrate through the medium of said emitter material layer;

removing by etching from the union of said first and second substrates said first substrate made of said single crystal material thereby exposing said oxide layer having disposed therein at least one protrusion possessing a sharp tip;

forming a gate electrode layer on said oxide layer;

removing said oxide layer and said gate electrode layer by etching thereby exposing the tip of emitter in at least

one protrusion covered by said oxide layer and said gate electrode layer and forming an opening part in the part of said gate electrode layer corresponding to said at least one protrusion; and

further removing by etching said oxide layer between said tip of emitter and said gate electrode layer in the opening part of said gate electrode layer thereby exposing the tip of emitter of said protrusion.

6. A method according to claim 5, further comprising the step of forming a conductive layer on said emitter material layer.

7. A method according to claim 5, wherein the union of said first substrate and said second substrate is attained by the technique of electrostatic bonding.

8. A method for the production of a field emission cathode structure comprising an emitter provided with a sharp point for emission of electrons and a controlling gate electrode, characterized by comprising a step of forming a first hole having a sharp pointed tip on a first (supporting) substrate, a step of forming an impurity diffusion layer on the surface of said first (supporting) substrate including said first hole, a step of forming an insulator layer on the surface of said impurity diffusion layer including said hole, a step of depositing an emitter material layer on the surface of said insulator layer including said hole while filling said hole with the emitter material, a step of integrally joining a second substrate to the surface of said emitter material layer, a step of removing by etching said first substrate thereby exposing the surface of said impurity diffusion layer provided with a projection corresponding to said first hole, and a step of selectively removing said impurity diffusion layer and said insulator layer thereby exposing a tip of the projection of said emitter material layer.

9. A method according to claim 8, wherein said impurity diffusion layer is formed as a gate electrode layer.

10. A method according to claim 8, which further comprises a step of forming a gate electrode layer on the surface of said impurity diffusion layer after the step of removing by etching said first supporting substrate thereby exposing the surface said impurity diffusion layer provided with a projection corresponding to said first hole and the step of selectively removing said impurity diffusion layer and said insulator layer thereby exposing the tip of the projection of said emitter material layer.

11. A method according to claim 8, wherein the integral union of said emitter material layer and said second supporting substrate is carried out by the electrostatic bonding method.

12. A method according to claim 8, wherein the formation of said insulator layer is effected by thermally oxidizing said impurity diffusion layer.

13. A method according to claim 8, wherein said impurity diffusion layer is formed by doping at least one element selected from the group consisting of B, Al, In, P, As, Ti, Ge, and Sn as an impurity into Si.

14. A method according to claim 13, wherein the concentration of said impurity is not less than  $3 \times 10^{19} \text{ cm}^{-3}$ .

15. A method for the production of a field emission cathode comprising an emitter provided with a sharp point for emission of electrons and a controlling gate electrode, characterized by comprising a step of forming a hole having a sharp point on a first supporting substrate, a step of forming an insulator layer on the surface of said first supporting substrate including said hole, a step of depositing an emitter material layer on the surface of said insulator layer including said hole while filling said hole with an emitter material, a step of integrally joining a second sup-

porting substrate to the surface of said emitter material layer, a step of etching said first supporting substrate through the exposed surface thereof until the end of a tip of the projection of said emitter material layer provided with the projection corresponding to said hole falls flush with the surface of said first supporting substrate after completion of said etching, and a step of selectively removing said insulator layer thereby exposing the tip of the projection of said emitter material layer.

16. A method for the production of a field emission cathode comprising an emitter provided with a sharp point for emission of electrons and a controlling gate electrode, characterized by comprising a step of forming an etching stopper layer on the first main surface of a first supporting substrate, a step of forming a hole having a sharp pointed tip 10 on said first main surface side of said supporting substrate through said etching stopper layer to a depth reaching

5 halfway along the thickness of said first supporting substrate, a step of forming an insulator layer on the surface of said etching stopper layer including said hole, a step of depositing an emitter material layer on the surface of said insulator layer including the hole while filling said hole with an emitter material, a step of integrally joining a second supporting substrate to the surface of said emitter material layer, a step of removing by etching said first supporting substrate from a second main surface side thereof until said etching stopper layer thereby exposing an end part of said insulator layer corresponding to said hole, and a step of selectively removing said insulating layer thereby exposing a tip of a projection of said emitter material corresponding to said hole.

\* \* \* \* \*